

## UNITED STATES PATENT OFFICE

2,243,980

## SOFTENING TEXTILES

Alfred Rheiner and Jakob Link, Basel, Switzerland, assignors to Sandoz Ltd., Basel, Switzerland

No Drawing. Application October 25, 1937, Serial No. 176,884. In Switzerland October 30, 1936

7 Claims. (Cl. 91—68)

It has been found that polyalkylenepolyamines acylated with high-molecular aliphatic carboxylic acids or the N-alkyl derivatives thereof in the form of their water-soluble salts are excellent softening agents for textiles of all kinds.

As acylated polyalkylenepolyamines products having the following general formula are used:



$\text{R}$  being a high molecular alkyl radical having at least 8 C-atoms.

$\text{R}_1$  and  $\text{R}_2$  being hydrogen or low molecular alkyl radicals with at most 4 C-atoms,

$n$  and  $m$  meaning whole numbers,

$Y$  representing hydrogen, a low molecular alkyl radical or any desired acyl radical and when  $m$  is greater than 1,  $Y$  may represent different substituents, whereby when  $Y$  represents acyl radicals, at least one  $Y$  must be hydrogen or an alkyl radical.

$X$  representing hydrogen or a low molecular alkyl radical or a high molecular acyl radical with at least 9 C-atoms.

Among polyalkylenepolyamines which are suitable as starting materials for the production of softening agents, the following may be mentioned: diethylenetriamine, triethylenetetramine, dipropylenetriamine, dibutylenetriamine and their derivatives partially alkylated at the N-atom.

The particularly effective polyacrylpolyamines can advantageously be prepared by allowing at least 2 molecular proportions of a fatty acid or one of its functional derivatives to act on 1 molecular proportion of a polyalkylenepolyamine. The polyacrylpolyamines thus obtained are therewith converted into water-soluble salts as for example the formate, acetate or lactate, and can be directly used in this form.

The treatment of textiles with the said agents is in general carried out in aqueous solution at 20–100° C., care being taken that the treating bath is always of neutral or weakly acid reaction. These softening agents are fully resistant to the hardness formers in normal water if about 25 ccm. of 10 per cent acetic acid or the equivalent quantity of formic acid or lactic acid etc., is added per 100 litres of bath and per degree of temporary hardness, to the hard water before use.

Cotton or artificial silk of all kinds thus treated in the skein or piece has a particularly smooth,

soft feel. Yarns become easily workable by such treatment.

Used as an addition to yarn dressings, in particular dressings for artificial silk, the described softening agents improve the winding and spooling qualities of the yarns and increase their elasticity and softness. In warp dressings they permit easy and rapid working on the loom.

The products also render valuable services in conjunction with the fillers usual in finishing, such as starch, dextrine, vegetable glue and the like, and they afford the finished material increased smoothness and softness.

The following examples illustrate the invention, the parts being by weight:

## Example 1

Mercerized cotton yarn is treated at 30–40° C. for ½ hour with an aqueous solution of 0.3 g. per liter of a softening agent obtained by the following method: 300 parts of a hardened train-oil are heated for 2–3 hours while stirring to 190° C. with 57 parts of diethylene triamine (water content about 5%), the water in the amine being distilled off. The yellowish coloured wax-like base thus obtained is then transformed as follows into the acetate: 1 part of the molten base at about 90° C. is mixed with 4 parts of equally hot acetic acid of 5% strength, the softening agent then being obtained as a paste easily soluble in hot water. The yarn treated therewith has a very soft, agreeable feel.

## Example 2

If instead of the product used in Example 1, the acetate of the base obtained according to Example 4 of the U. S. Patent No. 1,947,951 is used as softening agent, the goods treated therewith are again given a soft feel.

## Example 3

Skeins of artificial silk are treated at 30–40° C. with an aqueous emulsion of 4–5 g. per liter of a softening agent obtained in the following way: 314 parts of a hardened spermaceti-oil are heated with 43 parts of diethylenetriamine (water content about 8%) for 2½ hours, while stirring, to 190–195° C. During this heating 4 parts of an aqueous solution distill off. The resulting wax-like reaction product when mixed molten with hot dilute acetic or formic acid yields the softening agent as a milky emulsion of the higher alcohol formed in the reaction with the acetate or formate of the diacyl-diethylenetriamine. The skeins of artificial silk treated therewith have a very soft feel.

**Example 4**

A good cotton yarn dressing which gives the material treated at 70° C. a soft feel, is obtained if 100 g. of potato starch somewhat dissolved, 1 g. of glycerine and 3 g. of a softening agent obtained as described below, are used per liter of dressing.

284 parts of molten technical stearic acid at about 110° C. are mixed with 54 parts of diethylenetriamine and heated to 150° C. while stirring. With gradual temperature increase, at 150-190° C., 23 parts of an aqueous solution distill off, the last of which are best removed under reduced pressure. The base thus obtained, when converted into the acetate in a similar manner to that described in Example 1, yields the softening agent in paste form easily soluble in hot water.

A softening agent which can also be used as an addition to dressings is obtained by heating 213 parts of coco-nut oil with 57 parts of diethylenetriamine at 185-195° C. and subsequent conversion of the acylated base into the formate.

*Example 5*

A cotton fabric is treated at 70° C. in the padding machine (foulard) with a mixture of 80 g. of potato starch somewhat dissolved, 80 g. of dextrine, 60 g. of glucose and 2 g. of softening agent per liter of bath.

The so finished fabric in addition to good filling has a satisfactory softness. The softening agent used is prepared in the following manner. A mixture of 310 parts of castor oil and 54 parts of triethylenetetramine are maintained for about 3 hours while stirring at about 190° C. The base obtained, which has a consistency similar to wool grease, is converted with warm dilute acetic acid into the acetate which can be directly used as the softening agent.

In this example the corresponding oleic acid derivative can also be used as an addition to finishing dresses in a similar manner to the ricinoleic acid derivative.

### **What we claim is:**

1. A process of softening textiles, comprising treating same with water-soluble salts of diacylated polyalkylenopolyamines of the following general formula



- 10 R being a high molecular alkyl radical having at least 8 C-atoms, R<sub>1</sub>, R<sub>2</sub> and R<sub>3</sub> being one of the group consisting of hydrogen and low molecular alkyl radicals with at most 4 C-atoms, and n and m meaning whole numbers.

15 2. A process of softening textiles, comprising treating same with water-soluble organic salts of diethylenetriamine diacylated with technical stearic acid.

20 3. A process of softening textiles, comprising treating same with water-soluble organic salts of diethylenetriamine diacylated with the acids of hardened train-oil.

25 4. A process of softening textiles, comprising treating same with water-soluble organic salts of triethylenetetramine diacylated with the acids of castor oil.

30 5. A textile treating process wherein the textile is subjected to the softening action of a water-soluble acetate of diethylene-triamine which has been diacylated with technical stearic acid.

35 6. A textile treating process wherein the textile is subjected to the softening action of a water-soluble acetate of diethylene-triamine which has been diacylated with the acids of hardened train oil.

40 7. A textile treating process wherein the textile is subjected to the softening action of a water-soluble acetate of diethylene-triamine which has been diacylated with the acids of castor oil.

ALFRED RHEINER.  
JAKOB LINK.